

## UNITED STATES PATENT OFFICE

2,436,046

EMULSIFIABLE SOLUBLE OIL  
COMPOSITIONS

Norman E. Lemmon and Frederick W. Schuessler,  
Hammond, Ind., assignors to Standard Oil  
Company, Chicago, Ill., a corporation of  
Indiana

No Drawing. Application December 22, 1944,  
Serial No. 569,411

4 Claims. (Cl. 252—312)

1

This invention relates to improvements in sulfonic compounds and more particularly to the compounding of sulfonic acids possessing different solubility properties to produce a product having the desired oil and water solubilities.

In the refining of petroleum oils with sulfuric acid, particularly concentrated or fuming sulfuric acids, two types of sulfonic acids are formed; one type is preferentially water-soluble and is found in the acid sludge layer. These preferentially water-soluble sulfonic acids are of a greenish color and because of this characteristic color are known and referred to in the petroleum refining art as green sulfonic acids. The other type of sulfonic acids are preferentially oil-soluble and are found in the sulfuric acid treated oil. These preferentially oil-soluble sulfonic acids have a characteristic reddish-brown or mahogany color and are commonly referred to and identified as mahogany sulfonic acids. While these preferentially oil-soluble sulfonic acids or sulfonates from different stocks and by different acid treatments as a class are all soluble in oil, they all do not behave similarly in water solubility and/or emulsibility, that is, certain of the preferentially oil-soluble sulfonic compounds form relatively stable emulsions with water while other types of preferentially oil-soluble compounds do not form emulsions with water or are difficultly emulsifiable with water.

The mahogany sulfonic acids range in molecular weight from about 300 to about 600 and while they all are preferentially oil-soluble as compared to the green acids, their solubility in oil increases with increase in their molecular weights. The preferentially oil-soluble mahogany acids and the soaps thereof have found wide use in the preparation of emulsifiable petroleum products, such as in soluble cutting oils, drawing compounds, emulsifiable insect spray compounds, and in other fields such as in the preparation of anti-rust compounds, mineral aggregate coating agents, etc. For these various uses hydrocarbon sulfonic acids within the molecular weight range of from about 350 to about 550 have been found most

2

effective. The preferentially oil-soluble hydrocarbon sulfonic compounds having molecular weights above about 425 are of the type which are substantially water-insoluble or which are non-emulsifiable with water. Hereinafter and in the appended claims preferentially oil-soluble hydrocarbon sulfonic compounds, which term is used generically to include the sulfonic acids as well as the sulfonates which are preferentially oil-soluble but substantially non-emulsifiable with water, will be referred to as preferentially oil-soluble water non-emulsifiable sulfonic compounds. By the term "water non-emulsifiable" as used herein and in the appended claims is meant an oil-soluble sulfonic compound which does not pass the emulsion test described by F. M. Archibald in the article "Analysis of petroleum oil-soluble sulfonic acid soaps" on page 611 of the September 15, 1941, issue of the Analytical Edition of the Industrial and Engineering Chemistry.

Since in the refining of petroleum oils with sulfuric acid or other sulfonating agents, preferentially oil-soluble petroleum acids are obtained varying in molecular weight over a wider range than those which are most desirable for use in the compounding of various emulsifiable products, a large proportion of the preferentially oil-soluble petroleum sulfonic acids have found little utility and in many cases must be considered as waste by-products or used for inferior products. The most effective preferentially oil-soluble sulfonic acids for use in the compounding of emulsifiable products are those having molecular weights within the range of from about 350 to about 425. The sulfonic acids having molecular weights below about 350 possess such low oil-solubility properties that they are unsuited for this use, while the sulfonic acids having molecular weights above about 425 yield soaps which are so water-insoluble as to render them unsatisfactory for compounding in emulsifiable products. A method of modifying the water and oil-solubility properties of the sulfonic acids having molecular weights above about 425 to render

them satisfactory for use in emulsifiable compounds is therefore highly desirable.

It is an object of the present invention to provide a method of modifying the water- and oil-solubilities of soaps of sulfonic acids having molecular weights above about 425 to render such soaps satisfactory for use in the compounding of emulsifiable products. Another object of the invention is to provide a method for utilizing sulfonic acids having molecular weights above about 425 in emulsifiable products. Still another object of the invention is to prepare satisfactory emulsifiable products containing hydrocarbon sulfonic acids having molecular weights above about 425. Still another object of the invention is to provide a method of preparing soluble oil products utilizing hydrocarbon sulfonic acids having molecular weights above about 425. An additional object of this invention is to prepare soluble oil products containing hydrocarbon sulfonic acids having molecular weights above about 425. Other objects and advantages of this invention will become apparent from the following description thereof.

In accordance with the present invention sulfonic acids, particularly the hydrocarbon sulfonic acids, such as petroleum sulfonic acids; resulting from the treatment of petroleum oils with sulfonating agents, and having molecular weights above about 425 which normally are not satisfactory for use in the preparation of emulsifiable soluble oil products are made useful for this purpose by employing the soaps of such sulfonic acids in combination with water-soluble, detergent type soaps, such as, for example, water-soluble alkylated aromatic sulfonates, sulfates, etc. The quantity of the water-soluble detergent type soap employed will vary with the molecular weight of the preferentially oil-soluble hydrocarbon sulfonic acid soap employed. Stated in another way, the more water-insoluble preferentially oil-soluble hydrocarbon sulfonic acids require the addition of greater amounts of the water-soluble detergent type soaps. In general for the preparation of most emulsifiable soluble oil products employing preferentially oil-soluble water non-emulsifiable hydrocarbon sulfonic acid soaps require from about 0.5% to about 10% or more and preferably from about 1% to about 5% of water-soluble, detergent type soaps in order to obtain the satisfactory emulsifying properties.

In the refining of petroleum oils it is the general practice to treat the oils with concentrated or fuming sulfuric acid in increments of about  $\frac{1}{2}$  pounds of acid per gallon of oil. The sludge formed after each "dump" of acid is settled and withdrawn and the oil again treated with  $\frac{1}{2}$  pound of the acid per gallon of the oil. This treatment is continued until the oil has been refined to the desired degree. In the preparation of white oils such as those known as technical white oils and medicinal mineral oils, the oil is usually treated with a total of from about 3 to about 9 pounds of acid per gallon of oil.

The preferentially oil-soluble hydrocarbon sulfonic acids produced during each increment of acid treatment vary in molecular weight and relative oil solubility. In general, those sulfonates obtained from the acid treatment of a distillate of 100 to 300 seconds Saybolt Universal viscosity at 100° F. with 5 or more pounds of acid per gallon or from the treatment of a distillate of 300 to 900 or more seconds Saybolt Universal viscosity with 3 or more pounds of acid per gal-

lon, are water non-emulsifiable and unsatisfactory for use in the compounding of soluble oil products. These hydrocarbon sulfonic acids have molecular weights ranging from about 450 to 560. These hydrocarbon sulfonic acids cannot be satisfactorily used in the formulation of emulsifiable soluble oil products without modifying their properties with a water-soluble, detergent type soap, for example the alkylated aromatic sulfonates of the type hereinafter-described.

A method of obtaining these preferentially oil-soluble water non-emulsifiable sulfonic acid soaps which must be modified to make them suitable for use in soluble oil products is illustrated by the following example:

A petroleum oil distillate having a Saybolt Universal viscosity at 100° F. of about 200 seconds is treated with from about 7 to about 8 pounds of fuming sulfuric acid per gallon of oil in one-half pound increments or "dumps." After the acid sludge from each one-half pound acid "dump" is settled and withdrawn, the next one-half pound of fuming sulfuric acid is added to the oil. The temperature of the oil before the fuming acid is added thereto is maintained at a temperature below about 60° F. but due to the heat of reaction upon the addition of the sulfuric acid, the temperature of the oil may rise to from about 90° F. to about 100° F. After the required total amount of fuming sulfuric acid has been added to the oil and the oil freed of acid sludge, the acid-treated oil containing oil-soluble sulfonic acids dissolved therein, is neutralized with a solution of sodium hydroxide. The aqueous alkali solution is then separated from the oil solution containing dissolved therein sodium soap of sulfonic acids and the latter then separated from the oil by extraction with alcohol of about 60% strength. The alcohol layer containing dissolved sodium sulfonates is then separated from the oil and subsequently distilled to recover the alcohol and water. The sulfonic soap obtained in this manner contains from about 30% to about 60% sodium sulfonate, from about 30% to about 60% oil, from about 1% to about 10% water, and up to 10% of inorganic salts which may be removed by the procedure hereinafter-described.

The above procedure may be modified by separating the acid sludge from the acid treated oil, and extracting the oil with about 60% alcohol to remove the sulfonic acids, which may then be neutralized with sodium hydroxide and subsequently freed of the alcohol by distillation.

The crude soaps of these preferentially oil-soluble sulfonic acids obtained by the procedure described above may be freed of inorganic salts by purification. This purification is preferably accomplished by dilution of the crude soap with from about  $\frac{1}{2}$  to about 10 parts, preferably 1 to 2 parts of 50% or higher strength alcohol, preferably alcohol of 60 to 70% strength, and allowing the salts to settle while maintaining the mixture within the temperature range of 130 to 175° F., preferably 155 to 165° F. When the salts have settled the supernatant alcohol-soap layer is separated and the alcohol is recovered by conventional distillation procedure.

Preferentially oil-soluble water non-emulsifiable hydrocarbon sulfonic acids of this type are also obtained by treating a Kittrell distillate having a Saybolt Universal viscosity at 100° F. of from about 300 seconds to about 600 seconds in dumps of  $\frac{1}{2}$  pound of fuming sulfuric acid per gallon of distillate oil until a total of 3 to 4 pounds of acid per gallon of oil has been used. After

removal of the acid sludge the oil-soluble sulfonic acids are extracted from the oil with alcohol. Alcohol of from about 55% to about 70% and preferably of about 60% concentration can be used to extract the sulfonic acids, the amount of alcohol required for the extraction being within the range of from about 10 gallons to about 30 gallons of alcohol per 100 gallons of oil. The alcohol solutions of the preferentially oil-soluble hydrocarbon sulfonic acids are then treated such as by distillation to remove the alcohol. The soaps of the preferentially oil-soluble sulfonic acids so obtained are substantially as non-emulsifiable with water as are the preferentially oil-soluble sulfonic acid soaps obtained by treating petroleum distillates with 6 to 9 pounds of acid per gallon of oil, as above described; that is, these soaps are not suited for use in the formulation of oil-soluble products and must be modified by the addition of detergent type, water-soluble soaps before they can be used for this purpose. The preferentially oil-soluble water non-emulsifiable sulfonates obtained in the manner herein-described are typical of those of sulfonic acids having molecular weights above about 450 and which exhibit poor emulsifying properties.

Typical of the water-soluble detergent type soaps which are suitable as modifying soaps to render the preferentially oil-soluble water non-emulsifiable hydrocarbon sulfonic acid soaps of the type herein-described suitable components for the formulation of oil-soluble products are the alkylated aromatic sulfonic acid soaps in which the alkyl substituents contain from about 9 to about 17 and preferably from about 12 to about 16 carbon atoms in the alkyl groups. In the preparation of these alkylated aromatic sulfonic acid soaps an aromatic compound is alkylated by any suitable means and the alkylate sulfonated with a strong sulfonating agent such as sulfuric acid,  $\text{SO}_3$ , etc. The aromatic nucleus can be a monocyclic or polycyclic aromatic such as, for example, benzene, toluene, xylene, cumene, naphthalene, methyl naphthalene, ethyl naphthalene, isopropyl naphthalene, diphenyl, alkyl diphenyl, anthracene and alkyl anthracenes. The nucleus may contain in addition to the alkyl substituents halogen, nitro, hydroxy or other substituents. Suitable alkylating agents are olefin polymers, particularly those of ethylene, propylene, butylene and the like or mixtures thereof, preferably those having from about 9 to about 16 carbon atoms. Suitable olefin polymers are those having a distillation range of from about 320° to about 485° F. While it is preferable to alkylate the aromatic with an olefin polymer boiling within this distillation range, olefin polymers having a wider distillation range can be used and the alkylated aromatic fractionated to obtain a fraction having the desired distillation characteristics. The alkylation of the aromatic compound can be accomplished by reacting the aromatic and the alkylating agent in the presence of 90% to about 100% sulfuric acid, aluminum chloride, preferably activated with a trace of hydrogen chloride, hydrogen fluoride, boron fluoride, mixtures of hydrogen fluoride and boron fluoride, or other known alkylation catalysts. In addition to the olefin polymers, other suitable alkylating agents are haloparaffins, olefins, alkyl sulfates, aliphatic alcohols or aliphatic esters of wide molecular weight range.

Suitable water-soluble, detergent type sulfonates are the alkylated mono-nuclear aromatic sulfonates such as alkylated benzene or toluene

sulfonates having from about 9 to about 17, and preferably from about 12 to about 16 carbon atoms in the alkyl groups. Sulfonates of this type are suitably prepared by alkylating a mono-nuclear aromatic compound with an olefin polymer such as a propylene polymer or a butylene polymer of from about 9 to about 17 carbon atoms in the presence of sulfuric acid or aluminum chloride. The alkylated aromatic compound so obtained which contains from about 9 to about 17 carbon atoms in the alkyl groups is sulfonated with sulfuric acid of from about 88 weight percent to about 98 weight percent sulfuric acid. The reaction mass is then permitted to stratify and three strata are obtained. The lowest stratum comprises essentially spent sulfuric acid and alkylated aromatic sulfonic acids in which the alkyl groups contain less than about 9 carbon atoms and the upper strata comprises predominantly unsulfonated alkylated aromatics in which the alkyl groups contain more than about 17 carbon atoms and are of the type which upon sulfonation with suitable sulfonating agents would result in oil-soluble sulfonates. A middle stratum comprises predominantly the water-soluble, detergent type alkylated aromatic sulfonic acids. These alkylated aromatic sulfonates are suitable materials for modifying the emulsification characteristics of the preferentially oil-soluble and water non-emulsifiable hydrocarbon sulfonic acids of the type hereinbefore-described. The preparation of the water-soluble detergent type alkylated aromatic sulfonates suitable for the herein-described purpose is described in U. S. Patent 2,232,118, issued to L. P. Kyrides on February 18, 1941.

Suitable water-soluble, detergent type sulfonates are those prepared by the method described in U. S. 2,233,408, issued to L. H. Flett on March 4, 1941, and in U. S. Patent 2,218,472, issued to L. P. Kyrides on October 15, 1940. Other suitable water-soluble, detergent type materials suitable for the herein-described purpose are the soaps of sulfated or sulfonated fatty acids or alcohols known in the trade as surface-active agents. The preferentially oil-soluble water non-emulsifiable hydrocarbon sulfonates of the type described above possess certain desirable properties which if they could be incorporated in soluble oil type products would greatly increase the value of such products. Thus, for example, these sulfonates are very effective rust inhibitors and it would be highly desirable to incorporate them in soluble oil type products. However, because of their resistance to emulsification they cannot be satisfactorily employed in such products. However, by modifying these preferentially oil-soluble, water non-emulsifiable hydrocarbon sulfonates in the manner herein-described, they can readily be employed in soluble oil type products. The effect of adding small amounts of water-soluble, detergent type sulfonates to the preferentially oil-soluble, water non-emulsifiable hydrocarbon sulfonates is demonstrated by the following data which show the emulsification and rust inhibiting properties of a soluble oil base employing a preferentially oil-soluble, water non-emulsifiable mahogany sulfonate to which have been added various amounts of a water-soluble, detergent type sulfonate. The soluble oil base used was a mixture of 22% of a preferentially oil-soluble mahogany sulfonate having a molecular weight of about 450 to about 550, 3.5%

soda rosin soap and 74.5% of a light mineral oil having a Saybolt Universal viscosity of about 70 seconds at 100° F. The mahogany sulfonate was in a 50% oil solution. In making the test the soluble oil base was heated to 250° F. and 1 to 2% of a water or alcohol solution of a water-soluble detergent type soap added thereto. The water-soluble soap used in these tests was an alkylated aromatic sulfonate of about 9 to 15 carbon atoms in the side chains. In the table below the following rating is used:

- 5=good
- 4=passing specifications
- 3=questionable
- 2=not passing
- 1=poor

*Effect of addition of water-soluble detergent type sulfonate and diluent oil to soluble oil base formulated with a preferentially oil-soluble water non-emulsifiable mahogany sulfonate*

| Soluble Oil Base, parts | Adjuncts                          |               | Emulsion and Rust Rating             |                |        |                            |        |  |
|-------------------------|-----------------------------------|---------------|--------------------------------------|----------------|--------|----------------------------|--------|--|
|                         | Water-Soluble Sulfonate, per cent | Oil, per cent | Cold Water Emulsion Rating in 2% Sol | Rusting Rating |        | Room Temp. Emulsion Rating |        |  |
|                         |                                   |               |                                      | 2% Sol         | 4% Sol | 2% Sol                     | 4% Sol |  |
| 100                     | 0                                 | 0             | 4                                    | 5              | 5      | 2                          | 2      |  |
| 100                     | 0                                 | 20            | 1                                    | 5              | 5      | 3.5                        | 3.5    |  |
| 100                     | 1.0                               | 0             | 5                                    | 2              | 2      | 4                          | 4      |  |
| 100                     | 1.5                               | 0             | 5                                    | 5              | 5      | 3.5                        | 3.5    |  |
| 100                     | 1.5                               | 20            | 5                                    | 5              | 5      | 3                          | 3      |  |
| 100                     | 1.5                               | 30            | 2                                    | 5              | 5      | 4                          | 4      |  |
| 100                     | 2.0                               | 20            | 5                                    | 5              | 5      | 4                          | 4      |  |
| 100                     | 2.0                               | 30            | 3.5                                  | 5              | 5      | 4                          | 4      |  |

The addition of the hydrocarbon oil in the above test was used to show more clearly the effect of the water-soluble detergent type sulfonate in improving the emulsifying properties of the soluble oil base. The data show that as much as 20% to 30% of a hydrocarbon oil can be added to the soluble oil base in the presence of 2% of the water-soluble, detergent type sulfonate.

As stated above, the present invention is particularly adapted to the formulation of soluble oil products; for example, a composition comprising a hydrocarbon oil, from about 5% to about 11% of a preferentially oil-soluble, water non-emulsifiable petroleum sulfonate, from about 1% to about 5% of a water-soluble, detergent type soap such as, for example, an alkylated aromatic sulfonate having from about 9 to about 17 carbon atoms in the side chains and from about 1% to about 4% of a water-soluble soda soap of a carboxyl acid. The following example is illustrative of a soluble oil product formulation employing a preferentially oil-soluble water non-emulsifiable hydrocarbon sulfonate and a water-soluble detergent type soap. A soluble oil base is prepared by mixing 22% of a preferentially oil-soluble water non-emulsifiable mahogany soap (50% soap and 50% oil) with 3.5% soda rosin soap and 74.5% of a hydrocarbon oil having a Saybolt Universal viscosity at 100° F. of about 70 to 80 seconds and heating the mixture to a temperature of about 250° F. The mixture is then cooled and from about 1% to about 4% of a

water or alcohol solution of a water-soluble, detergent type sulfonate added to the mixture which is again reheated to a temperature of about 250° F. Alternatively the two types of sulfonates may be mixed and heated to about 250° F. and the rosin soap and the hydrocarbon oil then added to the heated mixture. If desired, from about 1% to about 3% of water and alcohol may be added to the soluble oil base to prevent phase separation in storage.

Although the present invention is particularly well adapted to the formulation of soluble oil bases, it is not limited to this particular use since we have found that the preferentially oil-soluble, water non-emulsifiable hydrocarbon sulfonates modified by the addition thereto of a water-soluble, detergent type sulfonate to give the proper water solubility are effective mineral aggregate coating agents. They can therefore be effectively used in bituminous materials such as road oils, asphalts and the like to form water resistant bituminous coatings on mineral aggregates.

While we have described our invention by reference to specific embodiments thereof, the invention is not intended to be limited thereto but includes within its scope such modifications as come within the scope of the appended claims.

We claim:

30. 1. A readily normally liquid soluble-oil composition comprising a major proportion of a hydrocarbon oil, from about 5% to about 11% of a sodium soap of a preferentially oil-soluble petroleum sulfonic acid having a molecular weight above about 450, which soap is normally unsuitable for use in soluble-oil compositions, from about 0.5% to about 10% of a water-soluble alkylated aromatic hydrocarbon sulfonate in which the alkyl substituents contain from about 9 to about 17 carbon atoms in the side chain and from about 1% to about 3% water.
35. 2. A readily emulsifiable normally liquid soluble-oil composition comprising a major proportion of a hydrocarbon oil, from about 5% to about 11% of a sodium soap of a preferentially oil-soluble water non-emulsifiable petroleum sulfonic acid having a molecular weight above about 450, which soap is normally unsuitable for use in soluble-oil compositions, from about 0.5% to about 10% of a sodium salt of an alkylated aromatic hydrocarbon sulfonic acid having from about 12 to about 16 carbon atoms in the side chain and from about 1% to about 3% water.
40. 3. A readily emulsifiable normally liquid soluble-oil composition comprising a major proportion of a hydrocarbon oil, from about 5% to about 11% of a sodium soap of a preferentially oil-soluble water non-emulsifiable petroleum sulfonic acid having a molecular weight above about 450 and which soap is normally unsuitable for use in soluble-oil compositions, from about 1% to about 5% of a water-soluble alkylated aromatic hydrocarbon sulfonate having from about 9 to about 17 carbon atoms in the side chain from about 1% to about 3% water.
45. 4. A readily emulsifiable normally liquid soluble-oil composition comprising a major proportion of a hydrocarbon oil, from about 5% to about 11% of a preferentially oil-soluble water non-emulsifiable petroleum sulfonic acid having a molecular weight of from about 450 to about 550, which soap is normally unsuitable for use in soluble-oil compositions, from about 1% to about 4% of a water-soluble soda rosin soap, from about 1% to about 5% of a water-soluble alkylated aro-

romatic hydrocarbon sulfonate having from about 9 to about 17 carbon atoms in the side chain from about 1% to about 3% water.

NORMAN E. LEMMON.  
FREDERICK W. SCHUESSLER.

## REFERENCES CITED

The following references are of record in the 10 Number  
file of this patent: 523,520

## UNITED STATES PATENTS

| Number    | Name      | Date          |
|-----------|-----------|---------------|
| 2,328,727 | Langer    | Sept. 7, 1943 |
| 2,205,950 | Flett     | June 25, 1940 |
| 2,265,799 | Carlson   | Dec. 9, 1941  |
| 2,314,450 | Holtzclaw | Mar. 23, 1943 |

## FOREIGN PATENTS

| Country       | Date          |
|---------------|---------------|
| Great Britain | July 16, 1940 |